

## UNITED STATES PATENT OFFICE

2,227,454

METHOD OF GOLD PLATING STEEL AND  
FERROUS ALLOYSJoseph B. Kushner, New York, N. Y., assignor to  
Benjamin Robinson, New York, N. Y.No Drawing. Application November 11, 1937,  
Serial No. 174,054

3 Claims. (Cl. 204—12)

This invention relates to an improved method for plating gold on steel and ferrous alloys, the object being to produce a method whereby gold may be plated directly on steel, iron, and other desired ferrous material in a way to be securely united with the article being plated.

In carrying out the invention it has been found that certain solutions hereinafter fully set forth must be used to properly cleanse a metal article 10 of oxide. It also has been found that the plating solution must contain a special reagent to inhibit the free acid remaining on the metal from attacking the surface of the metal during the plating operation.

When plating an article of steel or ferrous alloy, the article is first thoroughly cleaned of all oxide and is also etched to a certain extent, namely, until a fine etched surface is secured, so as to present an appreciably greater area to which 20 the gold may cling. More specifically, in carrying out the method the article is first cleansed in a suitable alkaline cleanser. The article is then dipped in a special bath to remove all oxide film from the cleansed article. The desired bath for 25 this purpose is set forth in the following formula:

## By volume

## Parts

|                                                                          |           |
|--------------------------------------------------------------------------|-----------|
| Hydrofluosilicic acid (concentrated),<br>H <sub>2</sub> SiF <sub>6</sub> | 50 to 100 |
| Hydrofluoric acid (35%), HF                                              | 5         |
| Water (distilled), H <sub>2</sub> O                                      | 25 to 50  |

A substitute for the acid hydrofluosilicic could be fluoroboric acid or the acids of the combination 35 of fluorine and the silicon earth group. Acids of this type, while sufficiently strong to destroy the oxide film on steel do not appreciably affect the under surface during a short exposure to them, and are therefore also suitable for the purpose of the present invention.

The article to be plated is dipped in the above 40 solution to secure the removal of the oxide film. This dipping operation may be from 30 seconds to 2 minutes according to the amount of etching desired as the solution will not only remove the 45 oxide film but will etch the surface of the article to be plated. This dipping may be done by ordinary dipping or current may be used and caused to pass through the article during the dipping 50 operation. This will produce a stronger etching effect.

After the article has been dipped as just described it is immediately immersed in clean water, which may be hot. After quickly dipping the 55 article in clean water it is immediately immersed

in the gold plating bath and the plating operation commenced. The preferable gold plating bath consists of the following ingredients in approximately the following proportions:

|                          | Grams |    |
|--------------------------|-------|----|
| Potassium cyanide        | 100   | 5  |
| Potassium carbonate      | 80    |    |
| Potassium gold cyanide   | 20    |    |
| Ammonium benzoate        | 2.5   |    |
| Sodium formate           | 2.5   | 10 |
| Water to make 10 liters. |       |    |

It will be noted that the ammonium benzoate and sodium formate are reagents and act to prevent too rapid plating. These inhibitors are desirable to cause a fine solid plating to be secured. It will therefore be seen that the formate and benzoate in the proportions set forth lower the 15 oxidizing effect of the free cyanide on the article being plated by depressing the CN ionization. The 20 gold has therefore the opportunity of being deposited on the surface of the article before a tarnish film can be formed on it.

As equivalents for the reagents and the other 25 gold plating salts the following could be used:

|                                |                                     |
|--------------------------------|-------------------------------------|
| KAuC <sub>2</sub>              | NaAu(CN) <sub>2</sub>               |
| or                             | NH <sub>4</sub> Au(CN) <sub>2</sub> |
| K <sub>2</sub> CO <sub>3</sub> | Na <sub>2</sub> CO <sub>3</sub>     |
| or                             | NH <sub>4</sub> CO <sub>3</sub>     |
| KCN                            | NaCN                                |
| or                             | NH <sub>4</sub> CN                  |
| Sodium formate                 | Potassium formate                   |
| or                             | Ammonium formate                    |
| Ammonium benzoate              | or                                  |
| Sodium                         | Potassium benzoate                  |

It will, of course, be understood that the article may be submerged in the plating bath as long as desired with the full current flowing. For an extremely light plating coat five or six 40 seconds would probably be satisfactory but usually the article is left in the bath for a longer time, as, for instance, one-half hour or longer with a current from 1 to 6 volts. As the surface is clean and is also formed with fine etching, the gold deposited on the article will interlock with the etched surface and form substantially an integral part thereof so that the plated article may be brushed or buffed, or polished in 45 any desired way and without becoming loose or 50 in any way injured.

I claim:

1. The method of electroplating gold on ferrous metals consisting in cleaning the article to be plated in an alkaline bath, subjecting the 55

- cleaned article to a solution of hydrofluosilicic acid until all oxide has been removed and an etched surface produced, washing the article in water after removal from the acid bath, and 5 then subjecting the article to an electroplating action in an electroplating bath containing potassium cyanide, potassium carbonate, potassium gold cyanide a reagent consisting of ammonium benzoate and sodium formate acting to 10 suppress the too rapid ionization of the gold so as to cause the gold to be deposited in a fine adherent state.
2. The method of plating gold on steel and ferrous alloy articles consisting in subjecting the 15 article to a mild ionized acid bath until all of the oxide on the article has been removed and the surface of the article has been attacked sufficiently to enlarge its surface by a very fine etched surface, washing the article in water and 20 immediately subjecting the article to an elec-

troplating action in a plating bath containing potassium cyanide, potassium carbonate, potassium gold cyanide and a reagent consisting of ammonium benzoate and sodium formate acting to cause the lowering of the attacking effect of the free cyanide on the article by depressing the ionization to permit the gold to be deposited on the surface of the article before a tarnish film can form. 5

3. The method of gold plating an article of 10 ferrous material on which an oxide film normally forms which includes subjecting the article to hydrofluosilicic acid until the oxide film has been removed and an etching operation has taken place to increase the surface, and electrolytically depositing a gold plate on the etched article from a cyanide plating bath containing ammonium benzoate and sodium formate. 15

JOSEPH B. KUSHNER. 20